

## UNITED STATES PATENT OFFICE.

HANS HOLZWARTH, OF MULHEIM, GERMANY.

## TURBINE BUCKET.

No Drawing.

Application filed August 23, 1921. Serial No. 494,643.

(GRANTED UNDER THE PROVISIONS OF THE ACT OF MARCH 3, 1921, 41 STAT. L., 1818.)

*To all whom it may concern:*

Be it known that I, HANS HOLZWARTH, a citizen of Germany, and resident of Mulheim, Germany, have invented certain new and useful Improvements in Turbine Buckets (for which I have filed applications in Germany, January 10, 1919; England, June 30, 1920, Patent No. 145,639; France, July 10, 1920, Patent No. 520,375; Holland, July 10, 1920; Italy, June 29, 1920), of which the following is a specification.

My invention relates to the construction of buckets for steam and gas turbines. The operative effects upon the buckets of large steam turbines operating at very high driving temperatures and particularly upon the buckets of gas turbines are entirely different from those upon the buckets of steam turbines of normal operation and moderate temperatures. In explosion turbines the force of the explosion upon the buckets is short and in the nature of a blow, so that said buckets must be of universal strength throughout. On the other hand, the centrifugal force which is developed requires the utmost economy in mass in the construction of such buckets. The high temperatures to which the first series of buckets in steam turbines and, above all, the buckets in gas or explosion turbines, are subjected, require the use of specially adapted material and that the strains be moderate in all parts thereof. The particular object of the present invention is to construct the buckets of a novel and efficient material specially adapted to meet and overcome the, in part, contradictory conditions set forth. My invention will be fully described hereinafter and the features of novelty will be pointed out in the appended claims.

The material which I use for constructing turbine buckets in accordance with the present invention comprises ingot iron, preferably practically unalloyed and free from objectionable and harmful mixtures and relatively poor in carbon and melted in an electric furnace or in a basic Martin furnace. The carbon content is preferably maintained below 0.1%, and in any case, should not materially exceed this point, and the percentage of manganese present therein ranges approximately from 0.30 to 0.50%;

nickel, chrome or other additions are not desirable. A material of the kind described, after a heat treatment at 450°, has a stretching or drawing limit of from 1300 to 1500 kg/cm<sup>2</sup>. If the calculable, permissible strains resulting from centrifugal force and bending forces do not exceed from 800 to 900 kg/cm<sup>2</sup>, the factor of safety is ample with a bucket of good form and a proper jet delivery.

Buckets constructed of the described material with the enumerated points in mind operate efficiently and maintain their form very satisfactorily during the operation of explosion turbines while other materials, and particularly alloyed ingot iron or alloyed steel, do not answer the requirements. In operation, the buckets of the turbine, when operated without water injection and only with air cooling, automatically become covered with a permanent protecting skin of ferrous oxide, that is to say, a combination of iron oxygen, which prevents rust and maintains the outer surface of the bucket permanently smooth and polished.

Various changes in the specific form described may be made within the scope of the claims without departing from the spirit of my invention.

I claim:

1. A bucket for gas and steam turbines adapted for high temperatures made of practically unalloyed iron having a low carbon content.

2. A bucket for gas and steam turbines adapted for high temperatures consisting of practically unalloyed iron having a low carbon content and free from nickel, chrome or other additions not including manganese.

3. A bucket for gas and steam turbines adapted for high temperatures consisting of practically unalloyed iron having a low carbon content and a manganese content ranging from about 0.30 to 0.50%.

4. A bucket for gas and steam turbines adapted for high temperatures made of practically unalloyed iron having a carbon content not exceeding 0.1%.

In testimony whereof I have hereunto set my hand.

HANS HOLZWARTH.